

# UNITED STATES PATENT OFFICE.

GEORGE P. KLINE, OF MOLINE, ILLINOIS.

## METALLIC COMPOSITION.

1,285,231.

No Drawing.

Specification of Letters Patent. Patented Nov. 19, 1918.

Application filed March 10, 1917. Serial No. 153,930.

*To all whom it may concern:*

Be it known that I, GEORGE P. KLINE, a citizen of the United States, residing at Moline, in the county of Rock Island and State of Illinois, have invented certain new and useful Improvements in Metallic Compositions, of which the following is a specification.

My invention relates to a new composition of metals, designed more specially for use in the construction of piston-rod packing, of that class for which Letters Patent of the United States No. 723681 were issued to me March 24, 1903. This packing is intended for use in and about locomotives and other engines in which the steam is used in a superheated condition. For this purpose it is necessary that the composition shall be of such a quality that it will comply with certain requirements. It must not be affected by the high degree of temperature which is possessed and imparted by said superheated steam; it must possess a sufficient degree of hardness to resist the frictional action of other parts having movement thereon; and it must not be so hard as to cause an abrasion of such movable parts.

My composition comprises copper, lead, and phosphorus, combined in substantially the following proportions, by weight, of the several ingredients, to wit: copper, eighty parts; lead, twenty parts; and phosphorus from one to two per cent. of the entire compound. The several parts are combined while in a molten state, and molded or otherwise formed into members or pieces of a desired pattern.

The phosphorus appears to assist in re-

taining the desired temper of the alloy of metals when exposed to extreme degrees of heat, such as is possessed by superheated steam. I am aware that phosphorus has been made use of before in the formation of alloys of metals, but not in the proportions named herein, nor with the results which are derived therefrom. The use of more than two per cent. of phosphorus is found to be unsatisfactory, and renders the compound useless for the purpose for which it is intended.

Any considerable variation in the proportions of copper and lead also renders the composition unfit for use in superheated localities, although when used with saturated steam the proportions could be changed to seventy parts of copper and thirty parts of lead, with proportional changes of such metals between said last named proportions and the proportions herein first set forth, to accord with varying steam pressures between the saturated and superheated conditions.

What I claim and desire to secure by Letters Patent, is—

The herein described composition of matter consisting of copper, eighty parts by weight, lead, twenty parts by weight, and phosphorus not to exceed two per cent. by weight of the total compound.

In testimony whereof I affix my signature in the presence of two witnesses.

GEORGE P. KLINE.

Witnesses:

W. N. HASKELL,  
ATEX NAECKEL.